# EUROPEAN PATENT SPECIFICATION

(11) **EP 0 322 763 B1**
(45) Date of publication and mention of the grant of the patent: **11.08.1993**
(21) Application number: 88121503.2
(22) Date of filing: 22.12.1988
(51) Int. Cl.: C21C 7/072, C21C 1/00, C22B 9/05

(54) **Method for cleaning molten metal and apparatus therefor**
Verfahren und Vorrichtung zum Feinen von Metallschmelzen
Procédé et appareillage de purification de métal liquide

(30) Priority: 25.12.1987 JP 326722/87; 25.12.1987 JP 326723/87; 12.01.1988 JP 3112/88; 12.01.1988 JP 3113/88
(43) Date of publication of application: 05.07.1989
(73) Proprietor: NKK CORPORATION, Tokyo (JP)
(72) Inventor: Ishii, Toshio c/o Patent & License and, Marunouchi Chiyoda-ku Tokyo (JP); Okubo, Yutaka c/o Patent & License and, Marunouchi Chiyoda-ku Tokyo (JP); Fukuda, Shuzo c/o Patent & License and, Marunouchi Chiyoda-ku Tokyo (JP)
(74) Representative: Füchsle, Klaus, Dipl.-Ing.

(56) References cited:
- CH-A- 420 237
- DE-A- 1 583 287
- DE-A- 1 903 212
- DE-B- 1 168 461
- DE-B- 1 433 406
- FR-A- 2 438 091
- GB-A- 1 048 895
- LU-A- 61 062

## Description

The present invention relates to a method for cleaning molten metal by removing inclusions suspended therein, and an apparatus therefor.

There have been proposed various methods for reducing the number of inclusions suspended in molten metal. Four such methods are described below:
(a) A first method, wherein inclusions in molten metal are trapped by gas bubbles produced by bubbling inert gas in molten metal at atmospheric pressure from the bottom of a vessel having molten metal therein. The inclusions are removed from the molten metal after the inclusions have risen to the surface of the molten metal.
(b) A second method, wherein inclusions in molten metal are removed by a filter made from calcium oxide which is put in a flow of the molten metal.
(c) A third method, wherein inclusions in molten metal are removed by throwing a solid such as calcium oxide capable of adsorbing the inclusions into the molten metal.
(d) A fourth method, wherein inclusions in molten metal are removed by having the inclusions risen to the surface of the molten metal or gone down by use of differences in densities of the inclusions.

However, to achieve manufacturing quality material, the total amount of oxygen in the molten metal needs to be limited to 15 ppm or less. When molten metal is cleaned by use of said methods, there can occur the following problems:

In the first method, a zone of the bubbling only spreads upwardly from a gas blowing-in inlet positioned at the bottom of a vessel. Moreover, there is a problem that it is difficult to bubble the molten metal from the whole vessel. When the bubbles produced by bubbling are large, the molten metal flows, bypassing the bubbles, during the bubbles' rising to the surface of the molten metal. In this case, micro-inclusions in the molten metal are hard to be trapped by the bubbles since the micro-inclusions also move together with the flow of the molten metal, bypassing the bubbles.

In the second method, when a filter capable of removing micro-inclusions is used, the filter often is choked and unable to be used soon after it has begun to be used.

In the third method, was the effectiveness of removing inclusions in molten metal by use of a solid such as calcium oxide diminishes, there occurs a necessity for withdrawing the solid out of the molten metal. In this case, there is a problem that the withdrawal of the solid is troublesome work and, moreover, the efficiency of the withdrawal of the solid is low.

In the fourth method, due to small particles of the micro-inclusions, the rising or the going-down of the micro-inclusions takes a lot of time. This leads to a decrease of the efficiency of removing the micro-inclusions.

It is an object of the present invention to provide a method for cleaning molten metal, wherein no only inclusions of an ordinary size, but also micro-inclusions can be removed from molten metal.

To accomplish said object, the present invention provides a method for cleaning molten metal as set forth in claim 1 below.

Preferred embodiments of the invention insofar as the method is concerned are defined in the dependant claims 2 to 9.

Further, the present invention provides an apparatus for cleaning molten metal, which comprises:
a first vessel which has an inlet for charging molten metal at the top end thereof and an outlet for discharging molten metal at the bottom thereof and in which the molten metal is pressurized by its hydrostatic pressure;
a second vessel which has an inflow port for pressurized molten metal at the bottom thereof and an outflow port for the pressurized molten metal and in which the pressurized molten metal goes upwardly and a pressure on the molten metal is reduced;
a communicating tube connecting the first vessel to the second vessel; and
a first bubbling device positioned at the bottom of the first vessel for bubbling the gas soluble in molten metal.

Preferred embodiments insofar as the apparatus is concerned are defined in the dependant claims 11 to 14.

The above objects and other objects and advantages of the present invention will now become apparent from the detailed description to follow, taken in connection with the appended drawings.
Fig.1 is a cross sectional view showing schematically an apparatus for cleaning molten metal by means of a batch process of the present invention;
Fig.2 is a cross sectional view illustrating another apparatus for cleaning molten metal by means of a batch process of the present invention;
Fig.3 is a cross sectional view showing schematically an apparatus for continuously cleaning molten metal with the use of a U-shaped vessel of the present invention;
Fig.4 is a graphic representation of a change in time of a total amount of oxygen in molten metal during processing the molten metal in example-1 and control-1;
Fig.5 is a cross sectional view showing schematically an outline of an apparatus used for a method of Preferred Embodiment-2;
Fig.6 is a graphic representation of the change of disturbance (flutter) of the surface of the molten metal, which was produced by applying static magnetic field to the molten metal, relative to magnetic flux density of static magnetic field in the abscissa;
Fig.7 is a cross sectional view illustrating an apparatus used for a method in Preferred Embodiment 3.
Fig.8 is a graphic representation of a change in time of a total amount of oxygen in molten metal during processing the molten metal in Example-4 of the present invention; and
Fig.9 is a cross sectional view illustrating an apparatus for continuously cleaning molten metal which is used in Example-5.

### Preferred Embodiment-1

The gas soluble in molten metal is bubbled in said molten metal under increased pressure. Inclusions of large particle size in the molten metal are trapped by the bubbles produced by a first bubbling, go upwardly to the surface of the molten metal and are removed. Since the molten metal under increased pressure is bubbled, a large amount of gas is uniformly dissolved in the molten metal by stirring the molten metal by means of bubbling. Thereafter, the gas dissolved in the molten metal is converted to fine gas bubbles when the pressure is rapidly reduced. The fine gas bubbles are produced from the whole area of the molten metal. Micro-inclusions are trapped by the fine gas bubbles, rise to the surface of the molten metal and are removed.

Nitrogen gas and hydrogen gas are selected as gases soluble in molten metal. Hydrogen gas is more desirable if the later removal of the gas having remained in the molten metal is taken into consideration. A gauge pressure of from 1 to 10 atm is preferred to the atmospheric pressure for applying a pressure on the molten metal. When the molten metal is pressurized at a pressure of less than 1 atm, it is less effective to pressurize the molten metal. When the molten metal is pressurized at a pressure of more than 10 atm, the apparatus becomes too expensive. The pressure on the molten metal is reduced in several stages from a pressure applied to the molten metal because fine bubbles are produced at every stage of the pressure reduction. For example, the pressure on the molten metal can be reduced as follows: 10 atm→ 7 atm → 4 atm → 1 atm. The method of the present invention described above can be carried out by means of a batch process wherein a pressure vessel is used, or a continuous process wherein a U-shaped vessel is used.

Fig.1 is a cross sectional view showing schematically an apparatus for cleaning molten metal by means of a batch process. A method for cleaning molten metal by means of the batch process will now be explained with specific reference to Fig.1. Firstly, molten metal is poured into pressure vessel 10. Thereafter, pressure vessel 10 is closed with cover 14 and the molten metal 12 is pressurized by the operation of a pressure valve 16 mounted on a duct connected to cover 14. Gas 20 soluble in the molten metal is blown in the molten metal under pressure from bubbling device 18 positioned at the bottom of vessel 10. After bubbling, the pressure applied to the molten metal 12 is rapidly reduced by further use of pressure valve 16. Finally, the inclusions which have risen to the surface of the molten metal are removed.

Fig.2 is a cross sectional view illustrating another apparatus for cleaning molten metal by means of _{,} a batch process. With the use of this apparatus, the pressure applied to molten metal 12 can be rapidly reduced by transferring the molten metal under pressure through communicating tube 22 to vessel 24 open to the air.

Fig.3 is a cross sectional view showing schematically a method for continuously cleaning molten metal with the use of a U-shaped vessel. Molten metal is continuously charged into a vessel through inlet 32 positioned at the top end of first vessel 30. Molten metal 12 goes down inside first vessel 30 and is gradually pressurized by its hydrostatic pressure. Molten metal 12 which has reached the bottom of vessel 30 is sufficiently pressurized by it hydrostatic pressure. There is an output port 34 at the bottom of vessel 30. The molten metal flows to communicating tube 36 through outflow port 34. the molten metal is bubbled by bubbling device 44 positioned at the bottom of first vessel 30 and by bubbling device 46 positioned at the bottom of communicating tube 36 connected to the first vessel. The molten metal, which has passed through communicating tube 36, enters second vessel 40 through inflow port 38 positioned at the bottom of second vessel40. There is output port 42 for discharging molten metal at the top end of second vessel 40. The molten metal rises toward outlet 42 for discharging molten metal inside second vessel 40. With the rise of the molten metal, the hydrostatic pressure on the molten metal is rapidly reduced, and gas dissolved in the molten metal appears in the molten metal as fine gas bubbles. The fine gas bubbles rise to the surface of the molten metal, trapping inclusions in the molten metal. The molten metal, which has gone out of outlet 42 for discharging molten metal from the second vessel 40, enters receptor 48. The inclusions floating on the surface of the molten metal inside receptor 48 are continuously removed.

### Preferred Embodiment-2

The use of Preferred Embodiment-1 is highly effective in removing inclusions in molten metal. In order further to reduce inclusion levels in the molten metal, it is good to decrease surface disturbance (flutter) of the molten metal, produced when the gas bubbles produced by bubbling, and the innumerable smaller bubbles produced by a pressure reduction, rise to the surface of the molten metal, in order that the inclusions which had risen to the surface of the molten metal could not mix again with the molten metal. Therefore, in a method of Preferred Embodiment-2, a static magnetic field is applied to the surface of the molten metal when the inclusions trapped by the bubbles produced by bubbling and by innumerable bubbles produced by the pressure reduction rise to the surface of the molten metal.

Fig.5 is a cross sectional view showing schematically an outline of an apparatus used for a method of Preferred Embodiment-2. When a static magnetic field is applied to the molten metal in a direction at right angles to the flow of the molten metal, a braking force against the flow of the molten metal takes place. Disturbance (flutter) of the molten metal surface just corresponds to an up-and-down flow of the molten metal bath. A force suppressing the up-and-down flow of the molten metal is produced by applying the static magnetic field to the surface of the molten metal with the use of electromagnet 50. Thereby, the amplitude of the disturbance is decreased, and this can prevent the occurrence of waves on the surface of the molten metal. Force F suppressing the flutter of the molten metal surface is represented by the following formula:

$\text{F = σ x B² x V}$

- σ :: electric conductivity of molten metal bath
- B:: magnetic induction
- V:: velocity of up-and-down movement of molten metal surface
The magnetic induction of the static magnetic field is preferred to be of from 0.1 to 0.5T (1000 to 5000 gauss). When said magnetic induction is less than 0.1T (1000 gauss), the force suppressing the flutter of the molten metal surface is small. When the magnetic induction exceeds 0.5T (5000 gauss), there is no change in the effectiveness of the force suppressing the flutter of the molten metal surface.

### Preferred Embodiment-3

The present inventor conducted various tests for the purpose of increasing the processing capability of the apparatus and concluded from them that, with a shortened processing time, micro-inclusions in the molten metal were not removed as expected. In consequence, it was thought to further increase the efficiency of removal of ordinary inclusions by the bubbling carried out before the pressure reduction process. As a result of later tests, it was concluded that the efficiency or removal of inclusions by bubbling could be increased by applying a low frequency electromagnetic force to the molten metal during bubbling and actively stirring the molten metal. It is thought that the efficiency of removal of inclusions is increased because the frequency with which inclusions in the molten metal strike against one another increases with stirring. The inclusions, having grown comparatively larger, rise to the surface of the molten metal during bubbling. In addition, since the amount of bubbling gas dissolved in the molten metal is to be expected to increase with stirring, a larger number of fine gas bubbles is created during the pressure reduction, and the efficiency in the removal of the micro-inclusions could be expected to be increased.

On the other hand, the temperature of the molten metal was reduced by the bubbling. In this connection, the amount of the bubbling gas dissolved in the molten metal is reduced. Fluidity of the molten metal is also reduced. In consequence, the effectiveness of the stirring effect of the bubbling is reduced.

In order to overcome those difficulties, the molten metal could be actively heated by Joule's heat produced by an induced current generated by applying a high frequency electromagnetic force to the molten metal during bubbling.

The reason why it was only during bubbling when the electromagnetic force was applied to the molten metal was the consideration that the inclusions, having once risen to the surface of the molten metal after the pressure reduction, should not thereafter be mixed again with the molten metal by electromagnetic stirring.

### Example-1

The cleaning of molten metal in Preferred Embodiment-1 was carried out by means of a batch process with the use of a pressure vessel of 2 m inside diameter and 3 m height as shown in Fig.1.

Firstly, 5 x 10⁴ kg (50 tons) of molten steel were poured into pressure vessel 10. Subsequently, pressure vessel 10 was closed with cover 14 and sealed. Atmospheric gas inside pressure vessel 10 was substituted for argon gas. Thereafter, a mixed gas consisting of 70% Ar gas and H₂ gas was bubbled in the molten steel for 20 minutes at a rate of 200 ℓ/min from bubbling device 18 positioned at the bottom of pressure vessel 10. A gas pressure inside pressure vessel was adjusted to 3 x 1.01325 x Pa (3 atm) by means of pressure valve 16. After the bubbling had finished, the gas pressure inside pressure vessel 10 was reduced to the atmospheric pressure by means of pressure valve 16. The molten steel was left as it was for 20 minutes until the gas bubbles produced by the pressure reduction rose to the surface of the molten steel. Finally, the molten steel was transferred to the next process.

The cleaning of molten steel was carried out as control-1 by use of a prior art gas bubbling method. That is, argon gas was blown in 5 x 10⁴ kg (50 tons) of the molten steel under the atmospheric pressure at a rate of 400 ℓ/min or 40 minutes.

Fig.4 is a graphic representation of a change in time of a total amount of oxygen in the molten steel during processing the molten steel in Example-1 and Control-1. The change of the total amount of oxygen in the molten steel in Example-1 is shown with a solid line and that in Control-1 with a dashed line. The total amount of oxygen before processing the molten steel was 80 ppm, but the amount of oxygen was decreased to 15 ppm in Example-1 while the amount of oxygen was decreased only to 30 ppm in Control-1. It was understood that the case of Example-1 of the present invention was superior to the case of Control-1 in the effectiveness of cleaning the molten steel. The total amount of bubbling gas was 16000 ℓ in Control-1. The total amount of the bubbling gas was 4000 ℓ ( 2800 ℓ of Ar gas and 1200 ℓ of H₂ gas ) in Example-1. In Example-1 of the present invention, the amount of gas used for the bubbling could be decreased and this could lead to a decrease of running cost.

### Example-2

A method of the present invention in Preferred Embodiment-1 was carried out by means of a continuous process with the use of a U-shaped vessel as shown in Fig.3. The dimensions of each portion of the vessel were as follows:

| | |
|---|---|
| Height of the first vessel: | 4 m |
| Inside diameter of the first vessel: | 1 m |
| Length of the communicating tube: | 2 m |
| Inside diameter of the communicating tube: | 30 cm |
| Bubbling device ( zones of 44 and 46 ) | 2 m |
| Diameter of the second vessel: | 10 cm |

Molten steel was continuously charged into the vessel from inlet 32 positioned at the top end of first vessel 30 at a rate of 2.5 x 10⁵ kg/hr (250 t/hr). A mixed gas consisting of 60% Ar gas and 40% H₂ gas was bubbled in the molten steel from bubbling devices 44 and 46 at a rate of 200ℓ/min. In consequence, the total amount of oxygen, which was 80 ppm before the molten steel was processed, was reduced to 12 ppm in the molten steel at the bottom of receptor 48. It was found that the effectiveness in oxidation of the molten steel became higher.

### Example-3

The cleaning of molten metal in Preferred Embodiment-2 was carried out by means of a batch process with the use of a pressure vessel of 2 m inside diameter and 3 m height as shown in Fig.5.

Molten metal was poured into pressure vessel 10 so that the level of the molten steel could rise to 2 m in height in pressure vessel 10. The atmosphere inside pressure vessel 10 was changed to argon gas. Thereafter, a mixed gas consisting of 70% Ar gas and 30% H₂ gas was blown in the molten steel from bubbling device 18 positioned at the bottom of pressure vessel 10 at a rate of 300ℓ/min to bubble the molten steel. A gas presure inside pressure vessel 10 was increased to 10 x 1.01325 bar (10 atm) during bubbling. Subsequently, a static magnetic field was applied to the surface of the molten steel bath by use of electromagnet 50. Thereby, a force suppressing flutter of the molten steel surface was produced. Thereafter, the bubbling was stopped. The gas pressure inside pressure vessel 10 was rapidly reduced by means of pressure valve 16, and fine gas bubbles were produced from the whole area of the molten steel. In Example-3, a static magnetic field was applied to the surface of the molten steel even when the gas pressure was reduced. Fig. 6 is a graphic representation of the change of the flutter of the molten steel surface, which was produced by applying a static magnetic field to the molten steel, relative to the magnetic flux density of the static magnetic field in the abscissa. In this schematic representation when the magnetic flux was over 0.1T (1000 gauss), there appeared an effect of suppressing flutter on the surface of the molten steel, and, when the magnetic flux exceeded 0.5T (5000 gauss), there was no change in the effectiveness of the force suppressing the flutter of the molten steel.

### Example-4

The cleaning of molten metal in Preferred Embodiment was carried out by means of a batch process with the use of a pressure vessel of 2 m inside diameter and 3 m height as shown in Fig.7.

Firstly, 5 x 10⁴ kg (50 tons) of molten steel were poured into pressure vessel 10. Subsequently, pressure vessel 10 was closed with cover 14 and sealed. Atmospheric gas inside pressure vessel 10 was changed to argon gas. Thereafter, mixed gas consisting of 70% Ar gas and 30% H₂ gas was blown in the molten steel from bubbling device 18 positioned at the bottom of pressure vessel 10 at a rate of 200 ℓ/min and the molten steel was bubbled for 20 minutes. A gas pressure inside pressure vessel 10 was adjusted to 3 x 1.01325 bar (3 atm) by means of pressure valve 16. An electromagnetic force was applied to the molten steel with the use of electromagnetic coils 52 arranged around pressure vessel 10 during bubbling,and the molten steel was subjected to electromagnetic stirring. Subsequently, the gas bubbling and the electromagnetic stirring were stopped, and the gas pressure inside pressure vessel 10 was reduced to atmospheric pressure by means of pressure valve 16. The molten steel was left as it was until the gas bubbles produced by the pressure reduction rose to the surface of the molten steel.

Fig.8 is a graphic representation of a change in time of a total amount of oxygen in the molten steel during processing the molten steel in Example-4. In Example-4, the totals amount of oxygen in the molten steel was already substantially reduced by an electromagnetic stirring during bubbling a mixed gas. It is thought that inclusions in the molten steel increasingly strike against one another, and that the inclusions having thereby grown comparatively larger rose to the surface of the molten steel, and that the total amount of oxygen in the molten steel was decreased. Moreover, the total amount of oxygen after the completion of all the processes also was decreased to 10 ppm, which was less than in Example-1. The decrease of the total amount of oxygen can be explained by the following two reasons: Firstly, comparatively small inclusions in the molten steel grew larger by striking against one another, being stirred during bubbling, and were easily trapped by gas bubbles; and, subsequently, the amount of gas dissolved in the molten steel became large and this increased the amount of fine gas bubbles produced during subsequent pressure reduction. Accordingly, it is necessary to take a little bit more time to leave the molten steel as it is after the pressure reduction so as to make the total amount of oxygen in the molten steel processed in Example-1 equal to the total amount of oxygen in the molten steel processed in Example-4.

### Example-5

A Preferred Embodiment of the apparatus for cleaning molten metal of the present invention will now be explained with specific reference to Fig.9. The apparatus for cleaning molten metal was composed of first vessel 30, communicating tube 36, second vessel 40 and vacuum storage vessel 56. First vessel was of 1 m inside diameter and of 5 m height. An opening at the top end of said first vessel was inlet 32 for charging molten metal. Outlet 34 for discharging molten metal was arranged at the bottom of first vessel 30. The molten metal flows through outlet 34 to communicating tube 36. Communicating tube 36 was of 50 cm inside diameter and of 6 m length. First bubbling device 44 was positioned at the bottom of first vessel 30 and second bubbling device 46 at the bottom of communicating tube 36 connected to first vessel 30 so that the molten metal could be bubbled from said bubbling devices 44 and 46. Gas storage chamber 54 was arranged at the position located a little bit beyond bubbling device 46 positioned at the bottom of communicating tube 36. Measures were taken by discharging a part of the bubbled gas to storage chamber 54 so that the gas bubbles rising to the surface of the molten metal inside second vessel 40, described later, could not grow too large. The gas inside gas storage chamber 54 was discharged by means of pressure valve 55. The molten metal, which had passed through communicating tube 36, entered second vessel 40 through inflow port 38 positioned at the bottom of second vessel 40. Second vessel 40 was of 30 cm inside diameter and of 5 m height. The inside diameter of second vessel 40 was made small so that the pressure on the molten metal could be rapidly reduced by having the molten metal flow more rapidly inside second vessel 40. Outlet 42 for discharging molten metal was positioned at the top end of second vessel 40. Vacuum storage vessel 56 of 2 m inside diameter connected to outlet 42 for discharging molten metal was arranged, and the molten metal stored in vacuum storage vessel 56 was degassed. Vacuum storage vessel 56 was arranged for the purpose of removing the gas bubbles produced by the bubbling and the pressure reduction, removing the inclusions rising to the surface of the molten metal, being trapped by the gas bubbles and discharging the gas dissolved in the molten metal even under atmospheric pressure. Gas in vacuum storage vessel 56 was exhausted by means of vacuum pump 57. Tube 58 of 30 cm inside diameter for bringing out the molten metal having been cleaned to the next process was connected to the bottom of vacuum storage vessel 56. In said apparatus,molten metal is continuously charged into a vessel through inlet 32 and the molten metal taken out through outlet 42 to vacuum storage vessel 56 can be the molten metal very well cleaned by bubbling the gas soluble in the molten metal from bubbling devices 44 and 46. That is, molten metal 12 discharged through inlet 32 is gradually pressurized by its own hydrostatic pressure, going down inside first vessel 30. A large amount of the gas bubbled from bubbling devices 44 and 46 dissolves in the molten metal.

Simultaneously, inclusions of ordinary size are trapped by bubbling gas and flow through communicating tube 36. A part of the bubbling gas enters gas storage chamber 54 and is taken out of gas storage chamber 54 upwardly by means of pressure valve 55. The molten metal having passed through communicating tube 36 enters second vessel 40 through inflow port 38 positioned at the bottom of second vessel 40. The pressure on the molten metal is rapidly reduced when the molten metal goes upwardly inside second vessel 40. Then, the gas dissolved in the molten metal appears as fine gas bubbles. Those fine gas bubbles rise to the surface of the molten steel, trapping inclusions in the molten metal. The molten metal enters vacuum storage chamber 56 through outlet 42. In vacuum storage vessel 56,the inclusions are trapped by the gas bubbles and the fine gas bubbles produced by the bubbling and the pressure reduction respectively and rise to the surface of the molten metal. To remove the gas soluble in the molten metal, the molten metal is degassed inside vacuum storage vessel 56. The molten metal cleaned by removing the soluble gas is taken out through passage 42.

The present inventor conducted a test of processing molten steel containing a total amount of 80 ppm of oxygen by use of the present apparatus. The molten metal was continuously charged into a vessel through inlet 32 at a rate of 2.5 x 10⁵ kg (250 t/hr). The molten metal was bubbled by a mixed gas consisting of 60% Ar gas and 40% H₂ gas blown in from bubbling devices 44 and 46 at a rate of 200 ℓ/min for 20 minutes. The molten metal containing a total amount of 12 ppm of oxygen was taken out via a vacuum storage device at a rate of 2.5 x 10⁵ kg/hr (250 t/hr) through passage 42.

## Claims

1. A method of removing inclusions from molten metal in which nitrogen and/or hydrogen is soluble, and comprising the steps of:
bubbling at least one of nitrogen and hydrogen gas into the molten metal whereby inclusions suspended in the molten metal are trapped and carried upwardly by the gas bubbles produced by bubbling, some of the gas also dissolving in the molten metal;
removing from the surface of the molten metal the inclusions carried upwards by the bubbles;
the method being characterised by the steps of:
pressurising the molten metal during the bubbling step, to a pressure in a range of from 1 to 10 x 1.01325 x 10⁵ Pa (1 to 10 atm) over atmospheric; and
reducing the pressure acting on the molten metal, after the bubbling step, to produce fine gas bubbles from solution in the molten metal, to trap and carry upwardly micro-inclusions suspended in the molten metal.

2. A method according to claim 1, characterized in that said pressure-reducing step is carried out in a plurality of successively lower pressure stages.

3. A method according to claim 1 or 2 characterized by applying static magnetic field to the surface of the molten metal when the inclusions trapped by the gas bubbles produced by bubbling in the bubbling process go upwardly, thereby to suppress disturbances of the molten metal surface.

4. A method according to claim 3, characterized in that said static magnetic field is one having a magnetic flux of from 0.1 to 0.5 T (from 1000 to 5000 gauss).

5. A method according to any one of claims 1 to 4, further comprising stirring the molten metal during bubbling in said bubbling process.

6. A method according to claim 5, characterized in that said stirring is by an electromagnetic force of low frequency.

7. A method according to any one of claims 1 to 6, characterized by heating the molten metal during said bubbling step.

8. A method according to claim 7, characterized in that said heating is by an electromagnetic force of high frequency.

9. A method according to any one of the preceding claims, further comprising vacuum degassing the molten metal.

10. Apparatus for cleaning molten metal, characterized by comprising
a first vessel (30) which has an inlet (32) for charging molten metal at the top end thereof and an outlet (34) for discharging molten metal at the bottom thereof and in which the molten metal is pressurized to above atmospheric pressure;
a second vessel (40) which has an inflow port (38) for the pressurized molten metal at the bottom thereof and an outflow port (42) for the molten metal and in which the pressurized molten metal goes upwardly and the pressure on the molten metal is reduced;
a communicating tube (36) connecting the first vessel to the second vessel; and
a first bubbling device (44) positioned at the bottom of the first vessel for bubbling the gas soluble in molten metal.

11. Apparatus as claimed in claim 10, further comprising a second bubbling device (46) in said communicating tube.

12. Apparatus as claimed in claim 10 or 11, further comprising a vacuum storage vessel (56) connected to the outlet for discharging molten metal which is arranged in said second vessel.

13. Apparatus as claimed in claim 10, 11 or 12, further comprising a gas storage chamber (54), by use of which a part of the bubbled gas is discharged.

14. Apparatus as claimed in any one of claims 10 to 13, characterized in that around said first vessel are electromagnetic coils for stirring molten metal in said first vessel.

## Patentansprüche

1. Verfahren zum Entfernen von Einschlüssen aus geschmolzenem Metall, in welchem Stickstoff und/oder Wasserstoff lösbar ist, und umfassend die Schritte:
Einperlen von mindestens Stickstoff- oder Wasserstoff-Gas in das geschmolzene Metall, wodurch im geschmolzenen Metall schwebende Einschlüsse eingefangen und von den durch Spülen erzeugten Gasblasen aufwärts getragen werden, wobei sich auch ein Teil des Gases im geschmolzenen Metall löst;
Entfernen der durch die Blasen aufwärts getragenen Einschlüsse von der Oberfläche des geschmolzenen Metalls;
wobei das Verfahren gekennzeichnet ist durch die Schritte:
Beaufschlagen des geschmolzenen Metalls während des Spülschrittes mit Druck bis auf einen Druck in einem Bereich von 1 bis 10 x 1,01325 x 10⁵ x Pa (1 bis 10 atm) über Atmosphärendruck; und
Verminderung des auf das geschmolzene Metall einwirkenden Drucks nach dem Spülschritt, um aus der Lösung im geschmolzenen Metall kleine Gasblasen zu erzeugen, um im geschmolzenen Metall schwebende Mikroeinschlüsse einzufangen und aufwärts zu tragen.

2. Verfahren nach Anspruch 1, dadurch gekennzeichnet, daß der besagte Druckminderungsschritt in einer Mehrzahl von Stufen mit sukzessiv geringerem Druck durchgeführt wird.

3. Verfahren nach Anspruch 1 oder 2, gekennzeichnet durch Beaufschlagung der Oberfläche des geschmolzenen Metalls mit einem statischen Magnetfeld, wenn die Einschlüsse aufsteigen, die von den durch Spülen beim Spülvorgang erzeugten Gasblasen eingefangen wurden, um dadurch eine Unruhe der Oberfläche des geschmolzenen Metalls zu unterdrücken.

4. Verfahren nach Anspruch 3, dadurch gekennzeichnet, daß das besagte statische Magnetfeld ein Magnetfeld mit einem magnetischen Fluß von 0,1 bis 0,5 T (von 1000 bis 5000 Gauß) ist.

5. Verfahren nach einem beliebigen der Ansprüche 1 bis 4, dadurch gekennzeichnet, daß es weiter ein Bewegen des geschmolzenen Metalls während des Spülens bei dem besagten Spülvorgang umfaßt.

6. Verfahren nach Anspruch 5, dadurch gekennzeichnet, daß das besagte Bewegen durch eine niedrigfrequente elektromagnetische Kraft erfolgt.

7. Verfahren nach einem beliebigen der Ansprüche 1 bis 6, gekennzeichnet durch Erhitzen des geschmolzenen Metalls während des besagten Spülschritts.

8. Verfahren nach Anspruch 7, dadurch gekennzeichnet, daß das besagte Erhitzen durch eine hochfrequente elektromagnetische Kraft erfolgt.

9. Verfahren nach einem beliebigen der vorhergehenden Ansprüche, dadurch gekennzeichnet, daß es weiter ein Unterdruckentgasen des geschmolzenen Metalls umfaßt.

10. Vorrichtung zum Reinigen von geschmolzenen Metall, dadurch gekennzeichnet, daß es umfaßt
einen ersten Behälter (30), der an seinem oberen Ende einen Einlaß (32) zum Beschicken mit geschmolzenem Metall und an seinem Boden einen Auslaß (34) zum Abziehen von geschmolzenem Metall besitzt, und in welchem das geschmolzene Metall bis über Atmosphärendruck mit Druck beaufschlagt wird;
einen zweiten Behälter (40), der an seinem Boden eine Einströmöffnung (38) für das unter Druck stehende geschmolzene Metall und eine Ausströmöffnung (42) für das geschmolzene Metall besitzt, und in welchem das unter Druck stehende geschmolzene Metall aufsteigt und der Druck auf das geschmolzene Metall vermindert wird;
ein Verbindungsrohr (36), das den ersten Behälter mit dem zweiten Behälter verbindet; und
eine am Boden des ersten Behälters angeordnete erste Spülvorrichtung (44) zum Einperlen des in geschmolzenem Metall lösbaren Gases.

11. Vorrichtung nach Anspruch 10, dadurch gekennzeichnet, daß sie weiter eine zweite Spülvorrichtung (46) in dem besagten Verbindungsrohr umfaßt.

12. Vorrichtung nach Anspruch 10 oder 11, dadurch gekennzeichnet, daß sie weiter einen Unterdrucklagerbehälter (56) umfaßt, der an dem Auslaß zum Abziehen von geschmolzenem Metall angeschlossen ist, welcher in dem besagten zweiten Behälter angeordnet ist.

13. Vorrichtung nach Anspruch 10, 11 oder 12, dadurch gekennzeichnet, daß sie weiter eine Gasspeicherkammer (54) umfaßt, durch deren Verwendung ein Teil des eingeperlten Gases abgeführt wird.

14. Vorrichtung nach einem beliebigen der Ansprüche 10 bis 13, dadurch gekennzeichnet, daß um den besagten ersten Behälter herum elektromagnetische Spulen zum Bewegen von geschmolzenem Material in dem besagten ersten Behälter angeordnet sind.

## Revendications

1. Procédé d'élimination d'inclusions dans un métal en fusion dans lequel l'azote et/ou l'hydrogène sont solubles, et comprenant les étapes consistant :
à faire barboter au moins un gaz choisi parmi l'hydrogène et l'azote gazeux, dans le métal en fusion, de sorte que les inclusions en suspension dans le métal en fusion, sont piégées et entraînées vers le haut par les bulles de gaz produits par le barbotage, une partie du gaz se dissolvant également dans le métal en fusion ;
à éliminer à partir de la surface du métal en fusion, les inclusions entraînées vers le haut par les bulles ;
caractérisé en ce qu'il comprend les étapes consistant :
à comprimer le métal en fusion au cours de l'opération de barbotage, jusqu'à une pression de 1 à 10 x 1,01325 x 10⁵ Pa (1 à 10 atm) au-dessus de la pression atmosphérique ; et
à réduire la pression s'exerçant sur le métal en fusion, après l'opération de barbotage, pour produire de fines bulles de gaz venues de solution dans le métal en fusion, afin de piéger et d'entraîner vers le haut les micro-inclusions en suspension dans le métal en fusion.

2. Procédé selon la revendication 1, caractérisé en ce que l'opération de réduction de pression est effectuée en plusieurs étapes sous pression successivement réduite.

3. Procédé selon la revendication 1 ou 2, caractérisé en ce qu'on applique un champ magnétique statique sur la surface du métal en fusion lorsque les inclusions piégées par les bulles de gaz produites par le barbotage dans l'opération de barbotage, montent de façon à supprimer les perturbations de la surface du métal en fusion.

4. Procédé selon la revendication 3, caractérisé en ce que le champ magnétique statique a un flux magnétique de 0,1 à 0,5 T (de 1 000 à 5 000 gauss).

5. Procédé selon l'une quelconque des revendications 1 à 4, caractérisé en outre en ce qu'on agite le métal en fusion en cours de barbotage dans ladite opération de barbotage.

6. Procédé selon la revendication 5, caractérisé en ce que l'agitation est effectuée sous l'effet d'une force électromagnétique à faible fréquence.

7. Procédé selon l'une quelconque des revendications 1 à 6, caractérisé en ce que l'on chauffe le métal en fusion au cours de l'opération de barbotage.

8. Procédé selon la revendication 7, caractérisé en ce que le chauffage est effectué à l'aide d'une force électromagnétique à haute fréquence.

9. Procédé selon l'une quelconque des revendications précédentes, caractérisé en outre en ce qu'on dégaze sous vide le métal en fusion.

10. Appareil pour épurer un métal en fusion, caractérisé en ce qu'il comprend :
un premier récipient (30) comportant un orifice d'entrée (32) pour charger un métal en fusion, à son extrémité supérieure, et un orifice de sortie (34) pour évacuer le métal en fusion, au fond de celui-ci, et dans lequel le métal en fusion est comprimé audessus de la pression atmosphérique ;
un deuxième récipient (40) comportant une ouverture d'entrée d'écoulement (38) pour le métal en fusion sous pression, au fond de celui-ci, et un orifice de sortie d'écoulement (42) pour le métal en fusion, et dans lequel le métal en fusion sous pression monte, et la pression exercée sur le métal en fusion est réduite ;
un tube de communication (36) reliant le premier récipient au deuxième récipient ; et
un premier dispositif de barbotage (44) disposé au fond du premier récipient, pour faire barboter le gaz soluble dans le métal en fusion.

11. Appareil selon la revendication 10, comprenant en outre un deuxième dispositif de barbotage (46) dans le tube de communication.

12. Appareil selon la revendication 10 ou 11, comprenant en outre un récipient de stockage sous vide (56) relié à l'orifice de sortie d'évacuation du métal en fusion disposé dans le deuxième récipient.

13. Appareil selon la revendication 10, 11 ou 12, comprenant en outre une chambre de stockage de gaz (54) à l'aide de laquelle une partie du gaz venu de barbotage, est évacuée.

14. Appareil selon l'une quelconque des revendications 10 à 13, caractérisé en ce que des enroulements électromagnétiques sont prévus autour du premier récipient, pour agiter le métal en fusion dans ce premier récipient.
